# EUROPEAN PATENT SPECIFICATION

(11) **EP 1 211 089 B1**
(45) Date of publication and mention of the grant of the patent: **27.12.2006**
(21) Application number: 01204419.4
(22) Date of filing: 19.11.2001
(51) Int. Cl.: B41M 5/00

(54) **Ink jet recording element and printing method**
Tintenstrahlaufzeichnungselement und -aufzeichnungsverfahren
Matériau d'enregistrement pour jet d'encre et procédé d'enregistrement

(30) Priority: 30.11.2000 US 726373; 30.11.2000 US 727227
(43) Date of publication of application: 05.06.2002
(73) Proprietor: EASTMAN KODAK COMPANY, Rochester, New York 14650 (US)
(72) Inventor: Landry-Coltrain, Christine J., c/o Estman Kodak Co, Rochester, New York 14650-2201 (US); Teegarden, David M., c/o Estman Kodak Company, Rochester, New York 14650-2201 (US)
(74) Representative: Haile, Helen Cynthia

(56) References cited:
- EP-A- 0 156 532
- EP-A- 0 409 440
- EP-A- 0 940 427
- WO-A-00/53405
- US-A- 4 542 059
- US-A- 5 374 475

## Description

This invention relates to an ink jet recording element, more particularly to a porous ink jet recording element and a printing method using the element.

In a typical ink jet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent. The solvent, or carrier liquid, typically is made up of water, an organic material such as a monohydric alcohol, a polyhydric alcohol or mixtures thereof.

An ink jet recording element typically comprises a support having on at least one surface thereof an ink-receiving or image-forming layer. The ink-receiving layer may be a porous layer which imbibes the ink via capillary action or a polymer layer which swells to absorb the ink.

Ink jet prints, prepared by printing onto ink jet recording elements, are subject to environmental degradation. They are especially vulnerable to water smearing and light fade. For example, since ink jet dyes are water-soluble, they can migrate from their location in the image layer when water comes in contact with the receiver after imaging. Highly swellable hydrophilic layers can take an undesirably long time to dry, slowing printing speed, and will dissolve when left in contact with water, destroying printed images. Porous layers speed the absorption of the ink vehicle, but often suffer from insufficient gloss and severe light fade. Porous layers are also difficult to coat without cracking. The support for the ink receiving layers is typically either porous or non-porous. When it is porous, the support itself can absorb non-imaging ink components such as water, solvents, and humectants, so that the ink receiving layer thickness can be minimized. However, when the support itself is non-porous, the ink receiving layer thickness must be great enough to absorb all the ink rapidly in order to prevent degradation of the image by dye smear during printing.

EP 940,427 discloses a method for making a microporous film for an ink jet recording element in which a hydrophobic polymer and a second hydrophilic polymer or copolymer of N-vinylpyrrolidone is dissolved in a certain solvent system, partially dried, and then washed to extract at least 50% by weight of the second polymer. The amount of the hydrophobic polymer to the second hydrophilic polymer is stated as 2:1 - 1:3. This reference also discloses the addition of a mordant to the polymer mixture. However, this reference does not disclose the use of a fluid-absorbing layer, so that the element has a problem in that it has a limited ink-absorbing capacity.

US-A-4,785,313 and US-A-4,832,984 disclose a two-layer ink jet receiving element wherein the layer adjacent the support is an image receiving layer and the outermost layer is an ink-transporting layer. However, there is a problem with this receiving element due to the fact that the ink-retaining layer is underneath the ink-transporting layer, which would scatter light, thus lowering the optical density.

US-A-5 374 475 discloses a record carrier for the receipt of coloring materials, including both inkjet and xerographic recordings. Membrane formation technologies, as known in the art, using a thermoplastic polymer in the porous layer, are generally referred to in column 2, lines 30-52.

EP-A-0 409 440 discloses an inkable sheet comprising an absorbent layer, which may be gelatin or be microporous, under an array of micropores in a surface zone forming a microporous layer having a pore density distribution such that the area occupied by micropores is from 5 to 30% of the exposed surface. This microporous layer on top of the absorbent layer is formed by a treatment of the surface of the absorbent layer with a modifying medium.

It is an object of this invention to provide an ink jet recording element which will provide improved ink uptake speed and capacity. Another object of the invention is to provide an ink jet recording element having a receiving layer that when printed upon has an excellent image quality. Still another object of the invention is to provide an ink jet recording element having a receiving layer wherein the printed image has improved water fastness. Yet still another object of the invention is to provide an ink jet recording element having improved ink absorbing capacity and drying rate when the support is non-porous or highly water resistant. Yet still another object of the invention is to provide a printing method using the above described element.

These and other objects are provided by the present invention comprising an ink jet recording element comprising a support having thereon in order:
a) a hydrophilic, fluid-absorbing layer, and
b) an image-receptive layer capable of retaining an ink jet image,
wherein the hydrophilic, fluid-absorbing layer has a thickness of 1 µm to 40 µm and the image-receptive layer has a thickness of 2 µm to 50 µm, the image-receptive layer comprising an open-pore membrane of a mixture of a water-insoluble polymer and a water-absorbent polymer, the mixture containing at least 25% by weight of the water-absorbent polymer,
the image-receptive layer being obtainable by dissolving the mixture of polymers in a solvent mixture, comprising at least one solvent which is a solvent for the water-insoluble polymer and at least one solvent with a higher boiling point which is not a solvent for the water-insoluble polymer, coating the dissolved mixture on the support and then drying to remove approximately all of the solvents to obtain the open-pore membrane.

By use of the invention, a recording element is obtained which will provide improved ink uptake speed and capacity, and when printed upon, has an excellent image quality and improved water fastness.

Another embodiment of the invention relates to an ink jet printing method comprising the steps of:
a) providing an ink jet printer that is responsive to digital data signals;
b) loading the printer with an ink jet recording element as defined above;
c) loading the printer with an ink jet ink composition; and
d) printing on the ink jet recording element using the ink jet ink in response to the digital data signals.

In order for the image-receptive layer of the invention to be sufficiently porous, the water-insoluble polymer must be coated from a solvent mixture combination such that an open-pore membrane structure will be formed when the solution is coated and dried, in accordance with the known technique of dry phase inversion. The formation of an open-pore membrane is accomplished by using a mixture of a good and poor solvent for the water-insoluble polymer. The poor solvent has a boiling point that is higher than that of the good solvent. When the solution is coated or cast onto a support and dried, the good solvent evaporates faster than the poor solvent, forming the membrane structure of the layer when the polymer phase separates from the solvent mixture. The open-pore structure results when the good solvent and poor solvent are removed by drying.

The water-insoluble polymer that can be used in the image-receptive layer of the invention may be, for example, a cellulose ester such as cellulose diacetate, cellulose triacetate, cellulose acetate propionate or cellulose acetate butyrate, cellulose nitrate, polyacrylates such as poly(methyl methacrylate), poly(phenyl methacrylate) and copolymers with acrylic or methacrylic acid, or sulfonates, polyesters, polyurethanes, polysulfones, urea resins, melamine resins, urea-formaldehyde resins, polyacetals, polybutyrals, epoxies and epoxy acrylates, phenoxy resins, polycarbonates, vinyl acetate polymers and copolymers, vinyl chloride-vinyl acetate copolymers, vinyl chloride-vinyl acetate-vinyl-alcohol copolymers, vinyl chloride-vinyl acetate-maleic acid polymers, vinyl chloride-vinylidene chloride copolymers, vinyl chloride-acrylonitrile copolymers, acrylic ester-acrylonitrile copolymers, acrylic ester-vinylidene chloride copolymers, methacrylic ester-styrene copolymers, butadiene-acrylonitrile copolymers, acrylonitrile-butadiene-acrylic or methacrylic acid copolymers, or styrene-butadiene copolymers. Cellulose ester derivatives, such as cellulose diacetates and triacetates, cellulose acetate propionate, cellulose acetate butyrate, cellulose nitrate, and mixtures thereof are preferred.

The water-absorbent polymer that can be used in the image-receptive layer of the invention may be, for example, polyvinylpyrrolidone and vinylpyrrolidone-containing copolymers, polyethyloxazoline and oxazoline-containing copolymers, imidazole-containing polymers, polyacrylamides and acrylamide-containing copolymers, poly(vinyl alcohol) and vinyl-alcohol-containing copolymers, poly(vinyl methyl ether), poly(vinyl ethyl ether), poly(ethylene oxide), hydroxyethylcellulose, hydroxypropylcellulose, hydroxypropylmethylcellulose, methylcellulose, and mixtures thereof. As noted above, the water-absorbent polymer is present in an amount of at least 25% by weight of said image-receptive layer. If the water-absorbent polymer is too high, for example, greater than 75% by weight, then the open pore membrane structure is not formed. If the water-absorbent polymer is less than 25% by weight, then poor image density is obtained.

The hydrophilic, fluid-absorbing layer useful in the invention may be gelatin, acetylated gelatin, phthalated gelatin, oxidized gelatin, chitosan, poly(alkylene oxide), a poly(vinyl alcohol), sulfonated polyester, partially hydrolyzed poly(vinyl acetate/vinyl alcohol), poly(acrylic acid), poly(1-vinyl pyrrolidone), poly(sodium styrene sulfonate), poly(2-acrylamido-2-methane sulfonic acid), polyacrylamide or mixtures thereof. In a preferred embodiment of the invention, the hydrophilic, fluid-absorbing layer is gelatin. In another preferred embodiment of the invention, the hydrophilic, fluid-absorbing layer is porous, comprising particulates such as an inorganic oxide or an organic polymer. For example, the porous, particulate-containing layer may be barium sulfate, calcium carbonate, clay, silica or alumina, or mixtures thereof.

In another preferred embodiment of the invention, the image-receptive layer contains at least 7% by weight of a mordant comprising a polymer or copolymer containing a quaternized nitrogen moiety. The mordant serves to improve the fixability of an ink jet image, thereby improving water fastness and smear. The mordant polymer can be a soluble polymer, or a crosslinked dispersed microparticle.

The mordant polymer or copolymer containing a quaternized nitrogen moiety which is useful in the invention can contain other comonomers such as, for example, styrenics, acrylates, imidazoles, vinylpyridines, etc. Examples of specific mordants include poly(styrene-co-1-vinylimidazole-co-1-vinyl-3-benzylimidazolium chloride), poly(styrene-co-1-vinylimidazole-co-1-vinyl-3-hydroxyethyl-imidazolium chloride), poly(styrene-co-1-vinylimidazoleco-1-vinyl-3-benzylimidazolium chloride-co-1-vinyl-3-hydroxyethylimidazolium chloride), poly(vinylbenzyltrimethylammonium chloride-co-divinylbenzene), poly(ethyl acrylate-co-1-vinylimidazole-co-1-vinyl-3-benzylimidazolium chloride), or poly(styrene-co-4-vinylpyridine-co-4-hydroxyethyl-1-vinylpyridinium chloride).

In a preferred embodiment of the invention, the quaternary nitrogen moiety is a salt of trimethylvinylbenzylammonium, benzyldimethylvinylbenzylammonium, dimethyloctadecylvinylbenzylammonium, 1-vinyl-3-benzylimidazolium, 1-vinyl-3-hydroxyethylimidazolium or 4-hydroxyethyl-1-vinylpyridinium. Preferred counter ions which can be used include chlorides or other counter ions as disclosed in US-A-5,223,338; US-A-5,354,813; and US-A-5,403,955. The hydrophilic, fluid-absorbing layer useful in the invention may also contain mordant polymers.

The choice of a good and poor solvent for the water-insoluble polymer will be effectively determined by the specific choice of polymer. The good solvent that can be used in the invention includes alcohols such as methanol, ethanol, n-propyl alcohol, isopropyl alcohol, isobutyl alcohol, Dowanol® solvents, glycols, ketones such as acetone, 2-butanone, 3-pentanone, cyclopentanone, and cyclohexanone, ethyl acetate, methylacetoacetate, diethylether, tetrahydrofuran, acetonitrile, dimethylformamide, dimethylsulfoxide, pyridine, chlorinated solvents such as methylene chloride, chloroform, carbon tetrachloride, and dichloroethane, hexane, heptane, cyclopentane, cyclohexane, toluene, xylenes, nitrobenzene, and mixtures thereof.

The poor solvent that can be used in the invention may be, for example, alcohols such as ethanol, n-propyl alcohol, isopropyl alcohol, isobutyl alcohol, 2-methyl-2,4-pentanediol, and Dowanol® solvents, glycols, ketones such as 2-butanone, 3-pentanone, cyclopentanone, and cyclohexanone, ethyl acetate, methylacetoacetate, diethylether, tetrahydrofuran, acetonitrile, dimethylformamide, dimethylsulfoxide, pyridine, chlorinated solvents such as carbon tetrachloride, and dichloroethane, hexane, heptane, cyclopentane, cyclohexane, toluene, xylenes, nitrobenzene, water, and mixtures thereof.

Since the image recording element may come in contact with other image recording articles or the drive or transport mechanisms of image recording devices, additives such as filler particles, surfactants, lubricants, crosslinking agents, matte particles and the like may be added to the element to the extent that they do not degrade the properties of interest.

Filler particles may be used in the open-pore membrane, the hydrophilic, fluid-absorbing layer, or both. Examples of filler particles are silicon oxide, fumed silica, silicon oxide dispersions such as those available from Nissan Chemical Industries and DuPont Corp., aluminum oxide, fumed alumina, calcium carbonate, barium sulfate, barium sulfate mixtures with zinc sulfide, inorganic powders such as γ-aluminum oxide, chromium oxide, iron oxide, tin oxide, doped tin oxide, alumino-silicate, titanium dioxide, natural or synthetic clay particles, organic particles, such as polystyrene matte beads, highly crosslinked organic polymer particles derived primarily from styrene, acrylates, or methacrylates, mixtures of these monomers, or mixtures with other monomers.

A dispersing agent, or wetting agent can be present to facilitate the dispersion of the filler particles. This helps to minimize the agglomeration of the particles. Useful dispersing agents include, but are not limited to, fatty acid amines and commercially available wetting agents such as Solsperse® sold by Zeneca, Inc. (ICI). Preferred filler particles are silicon oxide, aluminum oxide, calcium carbonate, and barium sulfate. Preferably, these filler particles have a median diameter less than 1.0 µm. The filler particles can be present in the amount from 0 to 80 percent of the total solids in the dried open-pore membrane layer, most preferably in the amount from 0 to 40 percent.

The open-pore membrane layer, the hydrophilic, fluid-absorbing layer, or both, may include lubricating agents. Lubricants and waxes useful either in the open-pore membrane layer or on the side of the element that is opposite the open-pore membrane layer include, but are not limited to, polyethylenes, silicone waxes, natural waxes such as carnauba, polytetrafluoroethylene, fluorinated ethylene propylene, silicone oils such as polydimethylsiloxane, fluorinated silicones, functionalized silicones, stearates, polyvinylstearate, fatty acid salts, and perfluoroethers. Aqueous or non-aqueous dispersions of submicron size wax particles such as those offered commercially as dispersions of polyolefins, polypropylene, polyethylene, high density polyethylene, microcrystalline wax, paraffin, natural waxes such as carnauba wax, and synthetic waxes from such companies as, but not limited to, Chemical Corporation of America (Chemcor), Inc., Michelman Inc., Shamrock Technologies Inc., and Daniel Products Company, are useful.

The open-pore membrane layer, the hydrophilic, fluid-absorbing layer, or both, may include coating aids and surfactants such as nonionic fluorinated alkyl esters such as FC-430®, FC-431®, FC-10®, FC-171® sold by Minnesota Mining and Manufacturing Co., Zonyl® fluorochemicals such as Zonyl-FSN®, Zonyl-FTS®, Zonyl-TBS®, Zonyl-BA® sold by DuPont Corp.; other fluorinated polymer or copolymers such as Modiper F600® sold by NOF Corporation, polysiloxanes such as Dow Coming DC 1248®, DC200®, DC510®, DC 190® and BYK 320®, BYK 322®, sold by BYK Chemie and SF 1079®, SF1023®, SF 1054®, and SF 1080® sold by General Electric, and the Silwet® polymers sold by Union Carbide; polyoxyethylene-lauryl ether surfactants; sorbitan laurate, palmitate and stearates such as Span® surfactants sold by Aldrich; poly(oxyethylene-co-oxypropylene) surfactants such as the Pluronic® family sold by BASF; and other polyoxyethylene-containing surfactants such as the Triton X® family sold by Union Carbide, ionic surfactants, such as the Alkanol® series sold by DuPont Corp., and the Dowfax® family sold by Dow Chemical.

The open-pore membrane layer, the hydrophilic, fluid-absorbing layer, or both, may include crosslinking agents, such as organic isocyanates such as tetramethylene diisocyanate, hexamethylene diisocyanate, diisocyanato dimethylcyclohexane, dicyclohexylmethane diisocyanate, isophorone diisocyanate, dimethylbenzene diisocyanate, methylcyclohexylene diisocyanate, lysine diisocyanate, tolylene diisocyanate, diphenylmethane diisocyanate; aziridines such as taught in US-A-4,225,665; ethyleneimines such as Xama-7® sold by EIT Industries; blocked isocyanates such as CA BI-12 sold by Cytec Industries; melamines such as methoxymethylmelamine as taught in US-A-5,198,499; alkoxysilane coupling agents including those with epoxy, amine, hydroxyl, isocyanate, or vinyl functionality; Cymel® crosslinking agents such as Cymel 300®, Cymel 303®, Cymel 1170®, Cymel 1171® sold by Cytec Industries; and bis-epoxides such as the Epon® family sold by Shell. Other crosslinking agents include compounds such as aryloylureas, aldehydes, dialdehydes and blocked dialdehydes, chlorotriazines, carbamoyl pyridiniums, pyridinium ethers, formamidinium ethers, and vinyl sulfones. Such crosslinking agents can be low molecular weight compounds or polymers, as discussed in US-A-4,161,407 and references cited.

In the present invention, the support can be either transparent or opaque. Opaque supports include plain paper, coated paper, synthetic paper, photographic paper support, melt-extrusion-coated paper, and laminated paper, such as biaxially oriented support laminates. Biaxially oriented support laminates are described in US-A-5,853,965; US-A-5,866,282; US-A-5,874,205; US-A-5,888,643; US-A-5,888,681; US-A-5,888,683; and US-A-5,888,714. These biaxially oriented supports include a paper base and a biaxially oriented polyolefin sheet, typically polypropylene, laminated to one or both sides of the paper base. Transparent supports include glass, cellulose derivatives, e.g., a cellulose ester, cellulose triacetate, cellulose diacetate, cellulose acetate propionate, cellulose acetate butyrate; polyesters, such as polyethylene terephthalate, polyethylene naphthalate, poly-1,4-cyclohexanedimethylene terephthalate, polybutylene terephthalate, and copolymers thereof; polyimides; polyamides; polycarbonates; polystyrene; polyolefins, such as polyethylene or polypropylene; polysulfones; polyacrylates; polyether imides; and mixtures thereof. The papers listed above include a broad range of papers, from high end papers, such as photographic paper to low end papers, such as newsprint.

The support used in the invention may employ an undercoat or an adhesive layer such as, for example, a vinylidene chloride-methyl acrylate-itaconic acid terpolymer or a vinylidene chloride-acrylonitrile-acrylic acid terpolymer. Other chemical adhesives, such as polymers, copolymers, reactive polymers or copolymers, that exhibit good bonding between the hydrophilic, fluid-absorbing layer and the support can be used. Other methods to improve the adhesion of the layer to the support include surface treatment such as by corona-discharge, plasma-treatment in a variety of atmospheres, UV treatment, etc, which is performed prior to applying the layer to the support.

The recording element of the invention can contain one or more conducting layers such as an antistatic layer to prevent undesirable static discharges during manufacture and printing of the image. This may be added to either side of the element. Antistatic layers conventionally used for color films have been found to be satisfactory, such as those in US-A-5,147,768. Preferred antistatic agents include metal oxides, e.g., tin oxide, antimony doped tin oxide and vanadium pentoxide. These antistatic agents are preferably dispersed in a film-forming binder.

The layers described above may be coated by conventional coating means onto a support material commonly used in this art. Coating methods may include, but are not limited to, wound wire rod coating, knife coating, slot coating, slide hopper coating, gravure coating, spin coating, dip coating, skim-pan-air-knife coating, multilayer slide bead, blade coating, curtain coating, multilayer curtain coating and the like. Some of these methods allow for simultaneous coatings of more than one layer, which is preferred from a manufacturing economic perspective if more than one layer or type of layer needs to be applied. The support may be stationary, or may be moving so that the coated layer is immediately drawn into drying chambers.

Ink jet inks used to image the recording elements of the present invention are well known in the art. The ink compositions used in ink jet printing typically are liquid compositions comprising a solvent or carrier liquid, dyes or pigments, humectants, organic solvents, detergents, thickeners, preservatives, and the like. The solvent or carrier liquid can be solely water or can be water mixed with other water-miscible solvents such as polyhydric alcohols. Inks in which organic materials such as polyhydric alcohols are the predominant carrier or solvent liquid may also be used. Particularly useful are mixed solvents of water and polyhydric alcohols. The dyes used in such compositions are typically water-soluble direct or acid type dyes. Such liquid compositions have been described extensively in the prior art including, for example, US-A-4,381,946; US-A-4,239,543 and US-A-4,781,758.

The following examples further illustrate the invention.

### Example 1 (Shows need for water-absorbent polymer in the image-receptive layer)

### Preparation of Element 1

### Preparation of the hydrophilic, fluid-absorbing layer HA-1:

A homogeneous solution was prepared from 8.25 wt. % pig-gelatin, 1.65 wt. % polyvinylpyrrolidone, PVP, (K90 from Aldrich Chemical Co.), and 1.1 wt. % of compound A-1 (see below) in distilled water, heated to 60 °C. The solution was metered to a slot-die coating apparatus and coated onto a moving base support comprised of a polyethylene resin-coated photographic paper stock, chill set at 4.5 °C, and dried at a temperature of 55 °C. The thickness of the HA-1 layer was measured to be about 10 ± 2 µm.

### Preparation of A-1

### Poly(vinylbenzyltrimethylammonium chloride-co-divinylbenzene)

In a 250 mL three-necked, round-bottomed header flask with a stopcock at the bottom and fitted with a mechanical stirrer, 100 mL of deionized, deaerated water, 15 g of dodecyl sulfate sodium salt, 101.5 g of vinylbenzyl chloride (mixture of 3- and 4-isomers), and 16.1 g of divinylbenzene (80%; mixture of isomers) were combined under nitrogen with stirring. The resulting emulsion was pumped through the stopcock over 90 min into a heated 1 L three-necked, round-bottomed reactor flask fitted with a mechanical stirrer, reflux condenser and nitrogen inlet, and containing 365 mL of deionized, deaerated water, 5.0 g of dodecyl sulfate sodium salt, 0.06 g of sodium metabisulfite, and 0.90 g of potassium persulfate. The reaction flask was maintained at 60 °C with constant stirring over the course of the polymerization. At the end of the monomer addition, an additional 0.03 g of g sodium metabisulfite, and 0.09 g of potassium persulfate were added to the reaction flask, and the polymerization was allowed to continue for an additional 60 min. Then the contents of the flask were cooled to room temperature.

Next, a solution of 93 g of sodium hydroxide in 175 ml of deionized water was added to the stirring latex. This was followed by the addition of a solution of 180 g of trimethylamine in 200 mL of isopropyl alcohol over approximately 60 min. This stirring reaction mixture was heated at 60°C for 24 hr. The reaction mixture was allowed to cool to room temperature and was dialyzed against deionized water to remove excess trimethylamine.

### Preparation of the open-pore membrane, image-receptive layer:

A homogeneous solution was prepared from 6 wt. % cellulose diacetate, CDA, (CA398-30, Eastman Chemical Company), 3 wt. % polyvinylpyrrolidone, PVP, (K25 from Aldrich Chemical Co.), 2 wt. % polymer M-1 (see below), 62.3 wt. % acetone (good solvent), and 26.7 wt. % 2-methyl-2,4,-pentanediol (poor solvent). The solution was coated onto layer HA-1 using a calibrated coating knife, and dried to remove substantially all solvent components to form a microporous membrane. The thickness of the dry microporous membrane layer was measured to be about 20 ± 2 µm.

### Preparation of M-1

Compound M-1 is a water-absorbent polymer and is a random copolymer of 1-vinylimidazole and ethyl acrylate and was synthesized as follows. A 3-L three-necked, round-bottomed flask fitted with a mechanical stirrer, reflux condenser and nitrogen inlet, was charged with 1200 g of N,N-dimethylformamide, 193.8 g of 1-vinylimidazole, and 206.2 g of ethyl acrylate. The solution was sparged with dry nitrogen for 30 min, and then 2.0 g of 2,2'-azobis(isobutyronitrile) was added and the flask was immersed in a 60°C constant temperature bath under a slight positive pressure of nitrogen and stirred for 24 hr. The polymer was precipitated into diethyl ether, filtered, and dried in vacuo for several days, resulting in an off-white solid.

### Preparation of Element 2

This element was prepared and coated the same as Element 1 except that the dry thickness of the dry microporous membrane, image-receptive layer was measured to be about 10 ± 2 µm.

### Preparation of Element 3

This element was prepared and coated the same as Element 1 except that the dry thickness of the dry microporous membrane, image-receptive layer was measured to be about 32 ± 2 µm.

### Preparation of Element 4

### Preparation of the hydrophilic, fluid-absorbing layer HA-2:

A homogeneous solution was prepared from 12 wt. % pig-gelatin in distilled water, heated to 60 °C. The solution was metered to a slot-die coating apparatus and coated onto a moving base support comprised of a polyethylene resin-coated photographic paper stock, chill set at 4.5 °C, and dried at a temperature of 55 °C. The thickness of the HA-2 layer was measured to be about 18 ± 2 µm.

### Preparation of the open-pore membrane, image-receptive layer:

A homogeneous solution was prepared the same as Element 1, coated over layer HA-2 using a calibrated coating knife, and dried to remove substantially all solvent components to form a microporous membrane. The thickness of the dry microporous membrane layer was measured to be about 34 ± 2 µm.

### Preparation of Element 5

### Preparation of the hydrophilic, fluid-absorbing layer HA-3:

This layer was prepared and coated the same as layer HA-2, except that the thickness of the dried layer was measured to be about 4 ± 2 µm.

### Preparation of the open-pore membrane, image-receptive layer:

A homogeneous solution was prepared and the same as Element 4, coated over layer HA-3 using a calibrated coating knife, and dried to remove substantially all solvent components to form a microporous membrane. The thickness of the dry microporous membrane, image-receptive layer was measured to be about 36 ± 2 µm.

### Preparation of Element 6

This element was prepared and coated the same as Element 5 except that the microporous membrane, image-receptive layer was prepared from 6 wt. % CDA, 3 wt. % PVP, (K25), 63.7 wt. % acetone, and 27.3 wt. % 2-methyl-2,4,-pentanediol, and the thickness of the dry microporous membrane, image-receptive layer was measured to be about 20 ± 2 µm.

### Preparation of Control Element C-1 (no water-absorbent polymer)

A homogeneous solution was prepared from 6 wt. % cellulose diacetate, CDA, 51.7 wt. % acetone (good solvent), and 42.3 wt. % 2-methyl-2,4,-pentanediol (poor solvent). The solution was coated onto layer HA-1 using a calibrated coating knife, and dried to remove substantially all solvent components to form a microporous membrane. The thickness of the dry microporous membrane layer was measured to be about 20 ± 2 µm.

### Printing

The above elements of Example 1 were printed using an HP Photosmart® Inkjet Printer and HP Photosmart® inks. The densities were read using an X-Rite 820® densitometer. The red channel density of the cyan patch at D-max (the highest density setting) and the green channel density of the magenta patch at D-max are reported in the following Table 1. The gloss of the top surface of the unprinted image was measured using a BYK Gardner gloss meter at an angle of illumination/reflection of 60°. The results are reported in Table 1 and are referenced to a highly polished black glass with a refractive index of 1.567 that has a specular gloss value of 100.

### Optical microscopy:

The location of the cyan and magenta dye in the printed samples of each element was determined as described below and is indicated in Table 1. Thin cross-sections (about 5 microns thick) of a D-max printed area in the sample were obtained using a Spencer A/O microtome. The sections were mounted on a glass slide with a drop of immersion oil, a cover slip was placed over the oil and sections were then pressed to disperse the oil. The slide was placed on a Jenaval Universal transmission microscope. The samples were examined for ink penetration and location. Magnifications up to 2500X can be used reliably.

**Table 1**

| Element | Polymers in image-receptive layer (Wt. Ratios) | Gloss 60 degree | D-max Cyan | D-max Magenta | Dye location |
|---|---|---|---|---|---|
| 1 | CDA/PVP/M-1 | 70 | 1.84 | 1.75 | open-pore membrane layer |
| | (55/27/18) | | | | |
| 2 | CDA/PVP/M-1 | 53 | 1.67 | 1.55 | open-pore membrane layer |
| | (55/27/18) | | | | |
| 3 | CDA/PVP/M-1 | 50 | 1.87 | 1.66 | open-pore membrane layer |
| | (55/27/18) | | | | |
| 4 | CDA/PVP/M-1 | 69 | 1.85 | 1.8 | open-pore membrane layer |
| | (55/27/18) | | | | |
| 5 | CDA/PVP/M-1 | 63 | 1.86 | 1.77 | open-pore membrane layer |
| | (55/27/18) | | | | |
| 6 | CDA/PVP | 54 | 1.98 | 1.71 | open-pore membrane layer |
| | (67/33) | | | | |
| Control C-1 | CDA (100) | 10 | 0.94 | 0.61 | HA-1 layer |

The above results show that the elements of the invention all had higher densities and surface gloss as compared to the control element. The above results also show that for all the elements of the invention, the dye is located in the open-pore membrane, image-receptive layer, rather than in the hydrophilic, fluid-absorbing layer.

### Example 2 (Shows need for at least 25 wt. % of water-absorbent polymer in the image-receptive layer)

### Preparation of Element 7

### Preparation of the hydrophilic, fluid-absorbing layer HA-4:

This layer was prepared and coated the same as layer HA-2, except that the thickness of the dried layer was measured to be about 10 ± 2 µm.

### Preparation of the open-pore membrane, image-receptive layer:

A homogeneous solution was prepared from 6 wt. % cellulose diacetate, CDA, 2 wt. % polyvinylpyrrolidone, PVP, (K25), 55.2 wt. % acetone (good solvent), and 36.8 wt. % 2-methyl-2,4,-pentanediol (poor solvent). The solution was coated onto layer HA-4 using a calibrated coating knife, and dried to remove substantially all solvent components to form a microporous membrane. The thickness of the dry microporous membrane layer was measured to be about 20 ± 2 µm.

### Preparation of Element 8

This element was prepared and coated the same as Element 7 except that Polymer M-1 was added at 3 wt. %, the PVP was 3 wt. %, the acetone was 52.8 wt. % and the 2-methyl-2,4,-pentanediol was 35.2 wt. %.

### Preparation of Element 9

This element was prepared and coated the same as Element 7 except that Polymer M-1 was added at 4 wt. %, the PVP was 4 wt. %, the acetone was 51.6 wt. % and the 2-methyl-2,4,-pentanediol was 34.4 wt. %.

### Preparation of Control Element C-2 (water-absorbent polymer less than 25 wt. %)

This element was prepared and coated the same as Element 7 except that the CDA was 6.4 wt. %, and the PVP was 1.6 wt. %.

### Preparation of Control Element C-3 (water-absorbent polymer less than 25 wt. %)

This element was prepared and coated the same as Element 7 except that the CDA was 6.8 wt. %, and the PVP was 1.2 wt. %.

### Preparation of Control Element C-4 (water-absorbent polymer less than 25 wt. %)

This element was prepared and coated the same as Element 7 except that the CDA was 7.2 wt. %, and the PVP was 0.8 wt. %.

### Preparation of Control Element C-5 (water-absorbent polymer less than 25 wt. %)

This element was prepared and coated the same as Element 7 except that the CDA was 7.6 wt. %, and the PVP was 0.4 wt. %.

### Printing

The above elements of Example 2 were printed using an HP Photosmart® Inkjet Printer and HP Photosmart® inks. Square patches of D-max (highest dye density) were printed onto the above elements. The density of each patch was read using an X-Rite 820® densitometer. Due to dye non-uniformity and poor quality of the printed control samples, the density of a one-inch-square D-max patch was averaged out and referenced to that obtained for a print on Kodak Inkjet Photo Paper, Catalogue No.800 6298, printed under the same conditions as the elements of Example 2. The relative % density of the cyan patch is defined as: $= \left[\left(Red channel average density of element\right)/(Red channel average density of Kodak Inkjet Photo Paper)\right] \times 100$ These values are reported in the following Table 2.

**Table 2**

| Element | Polymers in image-receptive layer (Wt. Ratios) | Total wt. % water-absorbent polymer | Relative % cyan at D-max |
|---|---|---|---|
| 7 | CDA/PVP (75/25) | 25 | 99 % |
| 8 | CDA/PVP/M-1 | 50 | 100 % |
| | (50/25/25) | | |
| 9 | CDA/PVP/M-1 | 58 | 100 % |
| | (42/29/29) | | |
| Control C-2 | CDA/PVP (80/20) | 20 | 71 % |
| Control C-3 | CDA/PVP (85/15) | 15 | 68 % |
| Control C-4 | CDA/PVP (90/10) | 10 | 47 % |
| Control C-5 | CDA/PVP (95/5) | 5 | 41 % |

The above results show that the elements of the invention all had a higher D-max as compared to the control elements with less than 25 wt. % water-absorbent polymer.

### Example 3 (shows improved waterfastness with a mordanting polymer)

### Preparation of Element 10

A homogeneous solution was prepared from 6 wt. % CDA, 3 wt. % PVP (K25), 2 wt % mordant polymer F-1 (see below), 53.4 wt. % acetone, and 35.6 wt. % 2-methyl-2,4,-pentanediol. The solution was coated onto layer HA-4 using a calibrated coating knife, and dried to remove substantially all solvent components to form a microporous membrane.

### Preparation of F-1

### Poly(styrene-co-1-vinylimidazole-co-1-vinyl-3-benzylimidazolium chloride- co-1-vinyl-3-hydroxyethylimidazolium chloride (50/35/5/10)

Poly(styrene-co-1-vinylimidazole) (50/50) was prepared in a semicontinuous solution polymerization at 54 wt.% solids in N,N-dimethylformamide (DMF) at 120 °C in a nitrogen atmosphere using Vazo 67® initiator from Du Pont Company as initiator. After a sample was removed for analysis, the remaining polymer solution was diluted to 20 wt.% in DMF to provide a stock solution for the preparation of mordant polymers.

Next, to a 1-L 3-necked round-bottomed flask equipped with a mechanical stirrer and a reflux condenser was added 625 g of the 20.0 wt. % solution of styrene-co-1-vinylimidazole in DMF. Benzyl chloride (8.0 g) was added, and the solution was stirred and heated at 100 °C under a slight positive pressure of nitrogen for 18 hr. A portion of the solution (25 g) was removed for analysis. Then, 9.7 g of 2-chloroethanol was added, and the solution was reheated with stirring at 100 °C for an additional 18 hr. The reaction mixture was cooled and the polymer was precipitated into diethyl ether with rapid stirring. The flaky precipitate was washed well with diethyl ether and dried in a vacuum oven.

### Preparation of Element 11

This element was prepared and coated the same as Element 10 except that Polymer F-1 was added at 0.6 wt. %, the acetone was 54.2 wt. % and the 2-methyl-2,4,-pentanediol was 36.2 wt. %.

### Preparation of Element 12

This element was prepared and coated the same as Element 10 except that Polymer F-1 was added at 0.2 wt. %, the acetone was 54.5 wt. % and the 2-methyl-2,4,-pentanediol was 36.3 wt. %.

### Printing and waterfastness test

The above elements of Example 3 were printed as in Example 2 using an HP Photosmart® Inkjet Printer and HP Photosmart® inks. Square patches of D-max (highest dye density) were printed onto the above elements. The density of each patch was read using an X-Rite 820® densitometer. Each patch was then submersed in distilled water for 5 minutes. After this watersoak, the density of each patch was once again read using an X-Rite 820® densitometer, and the % retained dye was calculated as follows: $% retained dye = \left(density after water test/density before water test\right) \times 100$ The results for the cyan patch and the magenta patch at D-max (the highest density setting) are reported in Table 3:

**Table 3**

| Element | Polymers (Wt. Ratios) | % retained cyan dye at D-max | % retained magenta dye at D-max | Observations after test |
|---|---|---|---|---|
| 8 | CDA/PVP/M-1 (50/25/25) | 93 | 69 | Severe dye smear |
| 10 | CDA/PVP/F-1 | 90 | 84 | Minimal dye smear |
| | (55/27/18) | | | |
| 11 | CDA/PVP/F-1 | 62 | 55 | Minimal dye smear |
| | (63/31/6) | | | |
| 12 | CDA/PVP/F-1 | 55 | 46 | Minimal dye smear |
| | (65/33/2) | | | |
| Control C-1 | CDA (100) | 22 | 26 | Measured density is very low even before watersoak |

The above results show that although Elements 8, 11, and 12 of the invention have reasonable waterfastness, compared to the control element C-1, the addition of a sufficient amount of mordant polymer F-1 improves the waterfastness of the printed image even more.

### Example 4 (shows improved ink dry time with the two layer structure on non-porous support, compared to a single layer structure, with no hydrophilic, fluid-absorbing layer)

### Preparation of Control Element C-6

The open-pore membrane, image-receptive layer solution was prepared as for Element 10 and the solution was coated onto a base support comprised of a polyethylene resin-coated photographic paper stock layer using a calibrated coating knife, and dried to remove substantially all solvent components to form a microporous membrane.

### Measurement of ink dry time:

A drop (about 0.5 microliter in size) of a magenta ink jet ink, prepared using a standard formulation with Dye 6 from US-A-6,001,161, was placed on each element and the time that it took for this spot to become dry to the touch was measured as the "ink drying time" as shown in the following Table:

**Table 4**

| Element | Hydrophilic, fluid-absorbing layer | Ink drying time |
|---|---|---|
| 10 | HA-4 (Gelatin) | 30 seconds |
| C-6 | none | 80 seconds |

The above results show that faster ink dry times can be achieved with the two-layer element of the invention as compared to the control element having only an open-pore membrane layer on a non-porous support.

### Example 5 (shows other hydrophilic, fluid-absorbing layer compositions) Preparation of Element 13

### Preparation of the hydrophilic, fluid-absorbing layer HA-5:

A homogeneous solution was prepared from 5 wt. % pig-gelatin, and 5 wt. % 0.7 µm particle size barium sulfate (Blanc Fixe Micro® from Sachtleben Corporation) in distilled water, heated to 60 °C. The solution was metered to a slot-die coating apparatus and coated onto a moving base support comprised of a polyethylene resin-coated photographic paper stock, chill set at 4.5 °C, and dried at a temperature of 55 °C. This is a filled layer but is not porous. The thickness of the HA-5 layer was measured to be about 8 ± 2 µm.

The open-pore membrane, image-receptive layer solution was prepared as for Element 10 and the solution was coated onto layer HA-5 using a calibrated coating knife, and dried to remove substantially all solvent components to form a microporous membrane.

### Preparation of Element 14

The open-pore membrane, image-receptive layer solution was prepared the same as Element 10 and the solution was coated onto a commercially available inkjet porous receiver paper containing a high amount of organic-inorganic hybrid fine particles, "Konica Photo IJ Paper QP ®", catalogue No. KJP-LT-GH-15-QP PI from Konica, using a calibrated coating knife, and dried to remove substantially all solvent components to form a microporous membrane.

### Printing

The above elements of Example 5 were printed as in Example 2 using an HP Photosmart® Inkjet Printer and HP Photosmart® inks. Square patches of D-max (highest dye density) were printed onto the above elements. The density of each patch was read using an X-Rite 820® densitometer.

The location of the cyan and magenta dye in the printed samples of each element was determined by optical microscopy, as described for Element 1 above. The following results were obtained:

**Table 5**

| Element | Hydrophilic, fluid-absorbing layer | D-max Cyan | D-max Magenta | Dye location |
|---|---|---|---|---|
| 10 | HA-4 (Gelatin) | 1.57 | 1.45 | Open-pore membrane layer |
| 13 | HA5 Gelatin/barium sulfate | 1.61 | 1.56 | Open-pore membrane layer |
| | (50/50) | | | |
| 14 | Konica QP Photo IJ ® paper | 1.71 | 1.64 | Open-pore membrane layer |

The above results illustrate that the hydrophilic, fluid-absorbing layer employed in the invention may also contain an inorganic filler.

## Claims

1. An ink jet recording element comprising a support having thereon in order:
a) a hydrophilic, fluid-absorbing layer, and
b) an image-receptive layer capable of retaining an ink jet image,
wherein the hydrophilic, fluid-absorbing layer has a thickness of 1 µm to 40 µm and the image-receptive layer has a thickness of 2 µm to 50 µm, the image-receptive layer comprising an open-pore membrane of a mixture of a water-insoluble polymer and a water-absorbent polymer, the mixture containing at least 25% by weight of the water-absorbent polymer,
the image-receptive layer being obtainable by dissolving the mixture of polymers in a solvent mixture, comprising at least one solvent which is a solvent for the water-insoluble polymer and at least one solvent with a higher boiling point which is not a solvent for the water-insoluble polymer, coating the dissolved mixture on the support and then drying to remove approximately all of the solvents to obtain the open-pore membrane.

2. The element of Claim 1 wherein the hydrophilic, fluid-absorbing layer is gelatin, acetylated gelatin, phthalated gelatin, oxidized gelatin, chitosan, poly(alkylene oxide), a poly(vinyl alcohol), sulfonated polyester, partially hydrolyzed poly(vinyl acetate/vinyl alcohol), poly(acrylic acid), poly(1-vinyl pyrrolidone), poly(sodium styrene sulfonate), poly(2-acrylamido-2-methane sulfonic acid), polyacrylamide or mixtures thereof.

3. The element of Claim 1 wherein the hydrophilic, fluid-absorbing layer is gelatin.

4. The element of Claim 1 wherein the hydrophilic, fluid-absorbing layer contains particulates.

5. The element of Claim 4 wherein the particulates comprise inorganic oxides or organic polymers.

6. The element of Claim 4 wherein the particulates comprise barium sulfate, calcium carbonate, clay, silica or alumina.

7. The element of Claim 1 wherein the water-insoluble polymer is a cellulose ester.

8. An ink jet printing method, comprising the steps of:
a) providing an ink jet printer that is responsive to digital data signals;
b) loading the printer with an ink jet recording element as defined in Claim 1;
c) loading the printer with an ink jet ink composition; and
d) printing on the ink jet recording element using the ink jet ink in response to the digital data signals.

## Patentansprüche

1. Tintenstrahlaufzeichnungselement mit einem Träger, auf dem in folgender Reihenfolge folgende Schichten angeordnet sind:
a) eine hydrophile, flüssigkeitsabsorbierende Schicht, und
b) eine Bildempfangsschicht, die ein Tintenstrahlbild aufzunehmen vermag,
worin die hydrophile, flüssigkeitsabsorbierende Schicht eine Dicke von 1 µm bis 40 µm aufweist und die Bildempfangsschicht eine Dicke von 2 µm bis 50 µm, wobei die Bildempfangsschicht eine offenporige Membran aus einer Mischung eines wasserunlöslichen Polymers mit einem wasserabsorbierenden Polymer umfasst und wobei die Mischung mindestens 25 Gew.-% des wasserabsorbierenden Polymers enthält,
und die Bildempfangsschicht durch Lösen der Polymermischung in einer Lösungsmittelmischung herstellbar ist, die mindestens ein Lösungsmittel umfasst, das ein Lösungsmittel für das wasserunlösliche Polymer ist, und mindestens ein Lösungsmittel mit einem höheren Siedepunkt, welches kein Lösungsmittel für das wasserunlösliche Polymer ist, sowie durch Auftragen der gelösten Mischung auf dem Träger und anschließendes Trocknen, um nahezu alle Lösungsmittel zu beseitigen und die offenporige Membran zu erzeugen.

2. Tintenstrahlaufzeichnungselement nach Anspruch 1, worin die hydrophile, flüssigkeitsabsorbierende Schicht Gelatine, acetylierte Gelatine, phthalatierte Gelatine, oxidierte Gelatine, Chitosan, Poly(alkylenoxid), ein Poly(vinylalkohol), sulfonierter Polyester, teilhydrolysiertes/teilhydrolysierter Poly(vinylacetat/-vinylalkohol), Poly(acrylsäure), Poly(1-vinylpyrrolidon), Poly(natriumstyrolsulfonat), Poly(2-acrylamid-2-methansulfonsäure), Polyacrylamid oder Mischungen daraus ist.

3. Tintenstrahlaufzeichnungselement nach Anspruch 1, worin die die hydrophile, flüssigkeitsabsorbierende Schicht Gelatine ist.

4. Tintenstrahlaufzeichnungselement nach Anspruch 1, worin die hydrophile, flüssigkeitsabsorbierende Schicht Partikeln enthält.

5. Tintenstrahlaufzeichnungselement nach Anspruch 4, worin die Partikeln anorganische Oxide oder organische Polymere enthalten.

6. Tintenstrahlaufzeichnungselement nach Anspruch 4, worin die Partikeln Bariumsulfat, Calciumcarbonat, Ton, Siliciumdioxid oder Aluminiumoxid enthalten.

7. Tintenstrahlaufzeichnungselement nach Anspruch 1, worin das wasserunlösliche Polymer ein Celluloseester ist.

8. Tintenstrahldruckverfahren mit folgenden Schritten:
a) Bereitstellen eines Tintenstrahldruckers, der auf digitale Datensignale anspricht;
b) Laden des Druckers mit einem Tintenstrahlaufzeichnungselement nach Anspruch 1;
c) Laden des Druckers mit einer Tintenstrahltintenzusammensetzung; und
d) Bedrucken des Tintenstrahlaufzeichnungselements mit der Tintenstrahltinte in Abhängigkeit von den digitalen Datensignalen.

## Revendications

1. Elément d'enregistrement à jet d'encre comprenant un support ayant sur celui-ci dans l'ordre :
a) une couche d'absorption de fluide hydrophile, et
b) une couche de réception d'image permettant de retenir une image à jet d'encre,
où la couche d'absorption de fluide hydrophile a une épaisseur de 1 µm à 40 µm et la couche de réception d'image a une épaisseur de 2 µm à 50 µm, la couche de réception d'image comprenant une membrane à pores ouverts d'un mélange d'un polymère insoluble dans l'eau et d'un polymère absorbant l'eau, le mélange contenant au moins 25 % en poids du polymère absorbant l'eau, la couche de réception d'image pouvant être obtenue en dissolvant le mélange de polymères dans un mélange de solvants, comprenant au moins un solvant qui est un solvant pour le polymère insoluble dans l'eau et au moins un solvant présentant un point d'ébullition plus élevé qui n'est pas un solvant pour le polymère insoluble dans l'eau, en appliquant le mélange dissous sur le support et en le séchant ensuite pour éliminer approximativement la totalité des solvants pour obtenir la membrane à pores ouverts.

2. Elément selon la revendication 1, dans lequel la couche d'absorption de fluide hydrophile est de la gélatine, de la gélatine acétylée, de la gélatine phtalatée, de la gélatine oxydée, du chitosane, du poly(oxyde d'alkylène), un poly(alcool vinylique), un polyester sulfoné, un poly(acétate de vinyle/alcool vinylique) partiellement hydrolysé, un poly(acide acrylique), une poly(1-vinylpirrolidone), un poly(sodium styrène sulfonate), un poly(acide sulfonique de 2-acrylamido-2-méthane), un polyacrylamide ou des mélanges de ceux-ci.

3. Elément selon la revendication 1, dans lequel la couche d'absorption de fluide hydrophile est de la gélatine.

4. Elément selon la revendication 1, dans lequel la couche d'absorption de fluide hydrophile contient des particules.

5. Elément selon la revendication 4, dans lequel les particules comprennent des oxydes inorganiques ou des polymères organiques.

6. Elément selon la revendication 4, dans lequel les particules comprennent du sulfate de baryum, du carbonate de calcium, de l'argile, de la silice ou de l'alumine.

7. Elément selon la revendication 1, dans lequel le polymère insoluble dans l'eau est un ester de cellulose.

8. Procédé d'impression à jet d'encre, comprenant les étapes consistant à :
a) fournir une imprimante à jet d'encre qui réagit à des signaux de données numériques,
b) charger l'imprimante avec un élément d'enregistrement à jet d'encre selon la revendication 1,
c) charger l'imprimante avec une composition d'encre pour jet d'encre, et
d) imprimer sur l'élément d'enregistrement à jet d'encre en utilisant l'encre pour jet d'encre en réponse aux signaux de données numériques.
